

Patented July 26, 1938

2,124,537

# UNITED STATES PATENT OFFICE

2,124,537

## MAGNESIUM BASE ALLOY

William O. Binder, Niagara Falls, N. Y., assignor  
to The Dow Chemical Company, Midland,  
Mich., a corporation of Michigan

No Drawing. Application April 24, 1937, Serial  
No. 138,738

5 Claims. (Cl. 75—168)

This invention relates to magnesium alloys and more particularly to those containing minor percentages of lead, manganese, and zinc.

One of the important problems confronting the magnesium industry is the production of magnesium alloys that possess good strength and related properties, good corrosion resistance, and good casting and fabricating characteristics. The commercial uses for which magnesium alloys 10 are suited depend in many instances on the availability of an alloy possessing two or more of the above mentioned characteristics.

The object of this invention is to prepare magnesium alloys that combine to a marked degree, 15 good physical properties, high corrosion resistance, and ease of casting and fabricating. Other objects and advantages will appear as the description proceeds.

My invention is based on the discovery that 20 highly desirable and useful alloys can be made from magnesium by alloying therewith approximately 0.5 to 22 per cent of lead, approximately 0.1 to 1.5 per cent of manganese, and approximately 0.5 to 10 per cent of zinc, and that such 25 alloys constitute a new product possessing highly desirable combinations of properties.

I have discovered that by adding zinc in amounts of about 0.5 to 10 per cent to the magnesium-manganese-lead alloys, new alloys are 30 produced whose physical properties are distinctly superior to the magnesium-manganese-lead alloys and that these new alloys are amenable to heat treatment, thereby resulting in still greater property improvement. This can be illustrated, 35 for example, by the addition of 2 per cent of zinc to the ternary magnesium+1.5 per cent of manganese+4 per cent of lead alloy and to the ternary magnesium+1.5 per cent of manganese+12 per cent of lead alloy.

### Properties of cast alloys

| 45                      | Composition | Tensile strength, lb./sq. in. | Yield strength, lb./sq. in. | Brinell hardness |
|-------------------------|-------------|-------------------------------|-----------------------------|------------------|
| Mg+1.5% Mn+4% Pb        | 18,400      | 4,200                         | 23.0                        |                  |
| Mg+1.5% Mn+4% Pb+2% Zn  | 22,500      | 5,200                         | 36.0                        |                  |
| Mg+1.5% Mn+12% Pb       | 20,000      | 5,000                         | 36.0                        |                  |
| Mg+1.5% Mn+12% Pb+2% Zn | 22,500      | 6,300                         | 38.6                        |                  |

The property improvements due to the presence of zinc in the heat treated alloys can be 55 illustrated by the following data:

### Properties of heat treated alloys

| 5                       | Composition | Tensile strength, lb./sq. in. | Yield strength, lb./sq. in. | Brinell hardness |
|-------------------------|-------------|-------------------------------|-----------------------------|------------------|
| Mg+1.5% Mn+4% Pb        | 19,600      | 5,200                         | 36.2                        |                  |
| Mg+1.5% Mn+4% Pb+4% Zn  | 22,600      | 7,500                         | 41.1                        |                  |
| Mg+1.5% Mn+4% Pb+6% Zn  | 26,900      | 10,700                        | 45.6                        |                  |
| Mg+1.5% Mn+12% Pb       | 19,500      | 5,500                         | 37.7                        |                  |
| Mg+1.5% Mn+12% Pb+4% Zn | 22,100      | 7,500                         | 44.3                        | 10               |

The typical property improvements in the heat treated and aged alloys were as follows:

### Properties of heat treated and aged alloys

| 15                      | Composition | Tensile strength, lb./sq. in. | Yield strength, lb./sq. in. | Brinell hardness |
|-------------------------|-------------|-------------------------------|-----------------------------|------------------|
| Mg+1.5% Mn+4% Pb        | 18,700      | 4,800                         | 36.8                        |                  |
| Mg+1.5% Mn+4% Pb+4% Zn  | 23,100      | 11,000                        | 46.9                        |                  |
| Mg+1.5% Mn+12% Pb       | 17,800      | 5,300                         | 37.7                        |                  |
| Mg+1.5% Mn+12% Pb+4% Zn | 22,900      | 13,500                        | 53.1                        |                  |

Another outstanding advantage of these new magnesium-manganese-lead-zinc alloys is that the above described property improvement has been obtained with little to no loss in corrosion resistance, particularly in the heat treated and heat treated and aged alloys. These alloys, therefore, possess excellent combinations of good physical properties and high corrosion resistance which make them valuable for many types of service.

### Corrosion resistance of Mg—Mn—Pb—Zn alloys in 3% NaCl solution for 1 week (mg/cm<sup>2</sup>/day)

| 40                      | Composition | Cast | Heat treated | Heat treated and aged |
|-------------------------|-------------|------|--------------|-----------------------|
| Mg+1.5% Mn+4% Pb        | 0.15        | 0.7  | 0.7          |                       |
| Mg+1.5% Mn+4% Pb+2% Zn  | 0.12        | 0.7  | 0.7          |                       |
| Mg+1.5% Mn+4% Pb+4% Zn  | 0.19        | 0.4  | 0.5          |                       |
| Mg+1.5% Mn+4% Pb+6% Zn  | 0.31        | 0.7  | 0.5          | 45                    |
| Mg+1.5% Mn+12% Pb       | 0.11        | 1.5  | 1.9          |                       |
| Mg+1.5% Mn+12% Pb+2% Zn | 0.97        | 1.1  | 1.4          |                       |
| Mg+1.5% Mn+12% Pb+4% Zn | 0.97        | 1.0  | 1.9          |                       |

The above alloys may be prepared by conventional methods of making magnesium alloys as by melting magnesium with a protective flux and adding thereto the respective alloying ingredients, either singly or simultaneously. Castings from my new magnesium alloys can be made in

conventional manner in dies or in molding sand containing oxidation inhibitors, such as ammonium fluoride compounds. For casting purposes, I normally prefer alloys containing 4 to 12 per cent of lead, 3 to 6 per cent of zinc, and 0.8 to 1.5 per cent of manganese. A recommended heat treatment consists of 16 to 18 hours at 790-840° F., while aging may be conducted at approximately 350° F. for 16 to 18 hours. It is often advantageous to give these alloys a preliminary heat treatment of 4 to 8 hours at approximately 650-700° F. prior to the above described heat treatment. Alloys for plastic deformation purposes should normally contain 1 to 6 per cent of lead, 0.5 to 1.5 per cent of manganese (preferably about 1.2 per cent), and of 0.5 to 3 per cent of zinc. Fabrication steps by plastic deformation operations are generally performed at 600-750° F.

20 Other modes of applying the principle of my invention may be employed instead of those explained, change being made as regards the ingredients and the steps herein disclosed, provided those stated by any of the following claims 25 or their equivalent be employed.

I particularly point out and distinctly claim as my invention:—

1. A magnesium-base alloy containing from about 0.5 to 22 per cent of lead, from about 0.1 to 1.5 per cent of manganese, and from about 0.5 to 10 per cent of zinc, the balance being magnesium.

2. A magnesium-base alloy containing from about 4 to 12 per cent of lead, from about 0.8 to 1.5 per cent of manganese, and from about 3 to 6 per cent of zinc, the balance being magnesium.

3. A magnesium-base alloy containing from about 1 to 6 per cent of lead, from about 0.5 to 1.5 per cent of manganese, and from about 0.5 to 3 per cent of zinc, the balance being magnesium.

4. A magnesium-base alloy containing about 12 per cent of lead, 1.5 per cent of manganese, and 4 per cent of zinc, the balance being magnesium.

5. A magnesium-base alloy containing about 4 per cent of lead, 1.2 per cent of manganese, and 2 per cent of zinc, the balance being magnesium.

WILLIAM O. BINDER. 25